

Feb. 9, 1954

K. A. FERN ET AL

2,668,667

Filed May 8, 1950

SEPARATION OF COARSE LIGHT MINERALS IN  
MULTIPLE CYCLONE-SEPARATOR STAGES

2 Sheets-Sheet 1



INVENTORS  
CHARLES F. ALLEN,  
K. A. FERN,

BY

*Robert Allen Morris*  
ATTORNEY

Feb. 9, 1954

K. A. FERN ET AL  
SEPARATION OF COARSE LIGHT MINERALS IN  
MULTIPLE CYCLONE-SEPARATOR STAGES

2,668,667

Filed May 8, 1950

2 Sheets-Sheet 2



INVENTORS  
CHARLES F. ALLEN,  
K. A. FERN,

BY  
Robert Hume Martin  
ATTORNEY

## UNITED STATES PATENT OFFICE

2,668,667

## SEPARATION OF COARSE LIGHT MINERALS IN MULTIPLE CYCLONE-SEPARATOR STAGES

Kenneth A. Fern, Johannesburg, Transvaal, Union of South Africa; and Charles F. Allen, Stamford, Conn., assignors to American Cyanamid Company, New York, N. Y., a corporation of Maine

Application May 8, 1950, Serial No. 160,772

13 Claims. (Cl. 241—24)

**1** This invention relates to an improved method of treating ores in which liberation of heavy minerals takes place at a fairly large size but the heavy minerals must be ground to a much finer size in order to separate their constituents or to treat them effectively.

The problem of grinding ores to release desired mineral values is a basic one in the ore dressing art. It is very common to grind in a closed circuit with a classifier, returning overflow or sands to the mill. This standard procedure is effective where all of the constituents are to be ground to approximately the same fineness, which is true in very many if not most ore grinding problems. There are, however, certain ores, particularly certain gold-bearing ores in South Africa and Canada, in which heavy minerals containing the gold, such as auriferous pyrite, can be liberated from the accompanying quartz or other siliceous gangue at a fairly coarse size. It is necessary, however, to grind the pyrite to a very fine size in order to set free the gold to a sufficient degree to permit effective economical recovery by cyanidation. Another type of ore is found in the class of pyritic copper ores where the copper and pyrite are liberated from the siliceous gangue at a comparatively large particle size, but require much finer grinding in order to separate the particles of the copper mineral from those of the pyrite.

In every case of these peculiar ores, for which the present invention is designed, ordinary closed circuit grinding is not satisfactory. If the grind is only sufficient to liberate metal values from the gangue, these are obtained in too coarse a particle size for effective treatment. On the other hand, if the grinding is down to the size at which the heavier mineral constituents are liberated from each other, or are made suitable for treatment, the power consumption for grinding becomes excessive and costs rise. In cases where the gangue tends to form slime, excessive slime formation also results, which introduces an additional severe problem.

According to the present invention, the problem is solved by the use of two stages of cyclone separation with autogenous medium in series together with a secondary grinding circuit. The cyclone separation is effected in conventional cyclones which operate with sufficient fine heavy material to act as a medium in cyclone separation, and the apparatus used therein is described in an article by Driessen "The Use of Centrifugal Force for Cleaning Fine Coal in Heavy Liquids and Suspensions with Special Reference to the Cyclone Washer" (The Journal of The Institute of Fuel, December 1945), and forms the subject

matter of U. S. Patent No. 2,543,689, issued February 27, 1951. Cyclone separation, as far as material of separable size is concerned, is on the basis of specific gravity differences, and is effected by centrifugal force. The materials to be separated, together with relatively fine heavy particles acting as a medium, are introduced tangentially under pressure into the cyclone near its base. Two vortices are formed, turning in the same direction, one passing down the cyclone to its apex, and the other up through a vortex finder in the base. Low specific gravity material is discharged through the base; high specific gravity material through the apex. The finely divided medium solids are discharged at both points. Throughout the remainder of the specification and claims, the term "cyclone" is used in this sense and this sense only.

The present process uses ordinary closed circuit grinding procedure on the feed. The ground material is classified in classifiers of conventional design, the underflow being returned to the mill, and the overflow, which may advantageously be 48 mesh or larger, is passed through the first cyclone separator. The vortex finder discharge, containing coarse and fine light material, normally gangue, and fine heavy medium particles, is introduced into a second cyclone separator. Relatively dilute vortex finder discharge from this second cyclone separator contains the light gravity material and some of the fine medium solids; and the apex discharge, which consists of somewhat thickened medium solids, is recirculated through the first cyclone. The material from the vortex discharge in the case of gold ores is ready for cyanidation, and in the case of multiple-mineral ores, such as pyritic copper ores, is subjected to suitable differential treatment, for example by flotation, if desired, after classification to remove coarse gangue.

The apex discharge of the first cyclone, which contains coarse heavy material and fine medium solids, is ground in a secondary mill of ordinary design, and then may be either recirculated through the first cyclone or may be mixed with the vortex finder discharge of the first cyclone and passed through the second cyclone. In either case the coarser heavy material is recirculated, being gradually reduced in size by the secondary mill until it finally leaves the system with the vortex finder discharge of the second cyclone.

The invention will be illustrated by the drawings, in which:

Figs. 1 and 2 are diagrammatic flowsheets of the process. The first flowsheet illustrates the modification in which the apex discharge from

the first cyclone, after being ground in the secondary mill, is mixed with the apex discharge of the second cyclone and recirculated through the first cyclone. Fig. 2 shows the alternative procedure, in which the ground apex discharge of the first cyclone is passed through the second cyclone.

It will be noted that a very marked reduction in grinding costs is obtained. The preliminary closed circuit grinding is carried only to the point where liberation of the heavy minerals from light gangue takes place. All of the light material is separated from the coarser heavy material in the first cyclone, and only the relatively smaller amount of the latter is ground to the small particle size necessary for liberation of the desired heavy mineral values. Only a small portion of the total ore is subjected to this fine grinding, with very great power savings.

The process has two other important advantages. First, the light material, such as gangue, is not ground to a fine size, with a resultant avoidance of excessive slime formation where slimy silicates are present. Secondly, the vortex finder discharge of the second cyclone contains only the finest of the heavy material.

The invention will be illustrated by typical examples of precious and base metal ores.

#### Example 1

A gold ore containing 1 oz. of gold per ton, mostly in the form of auriferous pyrite, assays approximately 10% sulfides and 90% siliceous gangue. This ore is treated by the process shown in Fig. 1, the overflow to the first cyclone containing siliceous gangue ground to -35 mesh. The vortex finder discharge from the second cyclone contains sulfides of a fineness of -325 mesh. This product is cyanided and produces a tailing residue having approximately the following composition:

| Cyanidation Residue   | Oz. Au/ton |
|-----------------------|------------|
| Siliceous Gangue..... | 0.015      |
| Sulfide Gangue.....   | 0.15       |
| Total Residue.....    | 0.028      |

As the sulfides constitute only 10% of the ore, the power required for grinding them to -325 mesh is a very small part of the total power.

A comparison test, using standard procedure, gives the following result: gangue ground to -65 mesh, sulfides to a nominal -150 mesh. Cyanidation gives the following result:

| Cyanidation Residue   | Oz. Au/ton |
|-----------------------|------------|
| Siliceous Gangue..... | 0.010      |
| Sulfide Gangue.....   | 0.30       |
| Total Residue.....    | 0.039      |

It will be noted that by the procedure of the present invention a much lower tailing is obtained with very materially less grinding cost. It is not practical by conventional processes to grind the siliceous gangue to only -35 mesh, as is the case with the process of Fig. 1, as this would result in excessive sulfide tailing residue losses.

#### Example 2

A copper ore containing sulfides of copper associated with pyrite and siliceous gangue, and containing approximately 1.5% copper, is treated by the process of Fig. 2. The overflow to the first cyclone contains siliceous gangue ground to

-48 mesh. The vortex finder discharge of the second cyclone contains the siliceous gangue together with sulfides of a fineness of approximately -325 mesh. This product is subjected to froth flotation using dicesyl dithiophosphoric acid as a promoter. A froth concentrate is obtained assaying approximately 25% copper, and a tailing assaying about 0.25% copper. The high grade of concentrate obtained is indicative of the excellent liberation of the copper minerals in the finely ground sulfides.

The above results were compared with an ordinary process of treating the same ore by grinding the siliceous gangue to -65 mesh, the sulfides, for the most part, being -100 mesh. When subjected to froth flotation under the identical conditions set forth above, a froth concentrate is obtained assaying just under 15% copper with a tailing of approximately 0.25% copper. It will be noted that by the process of the present invention a much higher grade concentrate is obtained with no increase in grinding costs. In fact, the power required is slightly less because of the relatively much larger amount of siliceous gangue as compared to the sulfides.

The flowsheets, which illustrate the operation of the process with autogenous medium, represent the preferred modification as the heavy minerals have to be ground in any event and their use as medium solids entails no additional expense. It is possible, of course, to introduce into either or both of the cyclones exogenous medium solids, such as finely divided ferrosilicon or similar magnetic material.

However, when exogenous media are used, medium cleaning devices must be introduced with additional equipment cost; therefore, while operative with exogenous media, the use of autogenous media is economically so much better that it constitutes the most practical embodiment of the invention.

#### We claim:

1. A method of preparing ore for recovery processes, the ore containing light minerals and the plurality of heavy minerals, the light minerals having a very much greater average particle size than the heavy minerals which comprises grinding the ore to approximately the relatively coarse particle size at which it is desired to reject the light minerals, subjecting an aqueous suspension of the ground ore to cyclonic separation in the presence of finely divided heavy medium solids in sufficient concentration to produce a separating gravity in the cyclone greater than the specific gravity of the fine minerals whereby a vortex finder discharge is produced containing the light minerals, both coarse and fine, associated with fine heavy mineral medium particles, and there is produced also an apex discharge containing heavy mineral only, subjecting the vortex finder discharge to a second cyclonic separation process at a gravity sufficiently high so that the light minerals are discharged through a vortex finder associated with very fine heavy mineral particles and there is produced an apex discharge containing only heavy mineral particles but of a particle size substantially coarser than the heavy mineral particles in the vortex finder discharge, grinding the apex discharge of the first cyclonic separation process and circulating at least a portion of said ground discharge through the second cyclonic separation process, recirculating the apex discharge from the second cyclonic separation process through the first as finely divided medium solids and removing

## 5

the vortex finder discharge from the second cyclonic separation in a form suitable for subjecting it to a separatory process capable of separating the very fine heavy mineral particles from the light particles.

2. A process according to claim 1 in which the ground apex discharge from the first cyclonic separation process is recirculated directly therethrough a portion of said ground material thereby being discharged through the vortex finder discharge of the first cyclonic separation process, and hence, subjected to the second cyclonic separation process.

3. A process according to claim 1 in which the ground apex discharge from the first cyclonic separation process is mixed with the vortex finder discharge of the same process and the mixture subjected to the second cyclonic separation process.

4. A process according to claim 1 in which the ore is a gold ore, the gold being associated with a heavy mineral fraction liberatable from light mineral gangue at a size approximating that at which the first cyclonic separation process is effected.

5. A process according to claim 4 in which the ground apex discharge from the first cyclonic separation process is recirculated directly therethrough a portion of said ground material thereby being discharged through the vortex finder discharge of the first cyclonic separation process, and hence subjected to the second cyclonic separation process.

6. A process according to claim 4 in which the ground apex discharge from the first cyclonic separation process is mixed with the vortex finder discharge of the same process and the mixture subjected to the second cyclonic separation process.

7. A process according to claim 1 in which the ore is a copper ore containing a plurality of copper minerals and the siliceous gangue separable from the copper-containing minerals at a particle size approximating that at which the first cyclonic separation process is carried out.

8. A process according to claim 7 in which the ground apex discharge from the first cyclonic separation process is recirculated directly there-

## 6

through a portion of said ground material thereby being discharged through the vortex finder discharge of the first cyclonic separation process, and hence, subjected to the second cyclonic separation process.

5 9. A process according to claim 7 in which the ground apex discharge from the first cyclonic separation process is mixed with the vortex finder discharge of the same process and the mixture subjected to the second cyclonic separation process.

10 10. A process according to claim 1 in which the liberation of the light minerals is effected by closed circuit grinding in series with a sizing device and the undersize of the sizing device is subjected to the first cyclonic separation process.

11 11. A process according to claim 1 in which the ore is a gold ore containing auriferous pyrite liberatable from light mineral gangue at approximately the particle size at which the first cyclonic separation is effected.

20 12. A process according to claim 11 in which the ground apex discharge from the first cyclonic separation process is recirculated directly therethrough a portion of said ground material thereby being discharged through the vortex finder discharge of the first cyclonic separation process, and hence, subjected to the second cyclonic separation process.

25 13. A process according to claim 11 in which the ground apex discharge from the first cyclonic separation process is mixed with the vortex finder discharge of the same process and the mixture subjected to the second cyclonic separation process.

KENNETH A. FERN.  
CHARLES F. ALLEN.

## References Cited in the file of this patent

## UNITED STATES PATENTS

| Number    | Name            | Date          |
|-----------|-----------------|---------------|
| 2,526,519 | Vogel-Jorgensen | Oct. 17, 1950 |

## OTHER REFERENCES

45 The Use of Centrifugal Force etc. by Driessen,  
The Journal of The Institute of Fuel, December  
1945.